

Aug. 10, 1937.

L. O. GARWIN

2,089,742

METHOD OF MELTING FINELY DIVIDED METAL

Original Filed Oct. 18, 1932 2 Sheets-Sheet 1



Fig. 1



Fig. 2

INVENTOR.

Louis O. Garwin

BY

Fay, Oberlin & Fay  
ATTORNEYS.

Aug. 10, 1937.

L. O. GARWIN

2,089,742

METHOD OF MELTING FINELY DIVIDED METAL

Original Filed Oct. 18, 1932 2 Sheets-Sheet 2



Fig. 3



Fig. 4



Fig. 5



Fig. 6



Fig. 7

INVENTOR.

Louis O. Garwin

BY

Fay, Oberlin Gray

ATTORNEY.

## UNITED STATES PATENT OFFICE

2,089,742

## METHOD OF MELTING FINELY DIVIDED METAL

Louis O. Garwin, Cleveland Heights, Ohio

Application October 18, 1932, Serial No. 638,291  
Renewed March 2, 1937

3 Claims. (Cl. 75—68)

The present invention, relating as indicated to a method of and apparatus for melting finely divided metal, is more particularly directed to a method and apparatus for melting finely divided aluminum scrap in even such finely divided form as borings, turnings, grindings and the like, converting this finely divided scrap material into pure metal or metal alloy and placing it in such condition that clean, sound castings may be made directly therefrom without employing any additional steps such as have heretofore been found necessary after the molten metal has been drawn off from the melting furnace.

To the accomplishment of the foregoing and related ends, said invention, then, consists of the means and steps hereinafter fully described and particularly pointed out in the claims; the annexed drawings and the following description setting forth in detail certain means and one mode of carrying out the invention, such disclosed means and mode illustrating, however, but one of the various ways in which the principle of the invention may be used.

In said annexed drawings:—

Fig. 1 is a central vertical section more or less diagrammatic in character of one form of my improved apparatus; Fig. 2 is a transverse section on the line 2—2 in Fig. 1; Fig. 3 is a horizontal section on the line 3—3 in Fig. 1; Fig. 4 is an end elevation of one of the end plates for the mold assembly shown in Fig. 2; Fig. 5 is a side elevation of the same; Fig. 6 is a plan view of one of the mold sections; and Fig. 7 is an end elevation of the same.

The melting of aluminum, aluminum alloys and analogous metals or metallic alloys presents certain problems which are not present in the handling of metals such as iron, brass and the like, in that these metals, which will hereinafter be referred to generally as aluminum, almost instantly oxidize and become coated with aluminum oxides when heated and exposed to the air. As a result of this characteristic it has been possible to remelt and use finely divided scrap aluminum only with considerable difficulty and under certain carefully maintained conditions. Even under these circumstances it has been found impossible to thoroughly clean the metal in the remelting furnace and additional operations have been carried out upon the metal following its withdrawal from the furnace in an attempt to more nearly approach the desired quality of the reworked material.

The equipment in use up to the present time for the remelting of finely divided aluminum has

possessed certain objectionable features and the furnaces with which I am familiar have required the use of a bath of molten material of unnecessarily large size, involving undue oxidation losses, increased labor costs and leaving the furnace available for less production time; and have produced harmful effects on the metal being melted by reason of permitting it to be in contact with the atmosphere at elevated temperatures or with fuel gases; and by having corners in which drosses collected to form nuclei for chemical and physical contamination; and by lacking proper means to adequately clean the molten metal by mechanical rupture of its inclusions therefrom; and by reason of the shape of the furnace chamber have allowed "freezing" of the contents at times and have made it extremely difficult to remove iron particles which invariably find their way into the bath and contaminate the aluminum. In addition to these objections the ordinary furnaces have, by reason of their shape, been uniformly subject to distortion in operation, and while this objection does not affect the operation of the furnace it has seriously affected the life of the furnace lining and the maintenance cost of the equipment.

The present invention is directed to a method and apparatus which avoid the difficulties heretofore met with, render it possible to rapidly and uniformly remelt and clean finely divided aluminum material in the furnace and withdraw completely purified, sound metal capable of being formed into desired cast shapes. Briefly stated, my improved method consists in charging into a furnace chamber containing a bath of clean, molten aluminum, additional finely divided aluminum, immersing the additional material in the bath, melting this material by heat conducted from a second chamber communicating with the first and also containing molten aluminum, and cleaning the said material from dirt, gases and other foreign material while maintaining an inert atmosphere over that portion of the furnace into which the additional finely divided material is charged to prevent oxidation, loss and inefficiency in the operation of the furnace. My method will be more clearly understood from reference to the furnace shown in the drawings, which are, however, more or less diagrammatic in character and not intended to illustrate the only form in which my improved apparatus can be embodied.

Referring now to Fig. 1, there is shown a furnace 1 consisting of an outer retaining sheet 2 of metal and an inner refractory lining 3 which

5

10

15

20

25

30

35

40

45

50

55

may conveniently be formed of plastic refractory material formed or plastered against the outer retaining shell of a sufficient depth to provide a lining of suitable characteristics for the melting 5 of such materials as aluminum and other light metals to which the present process is adapted. The furnace is formed with a slightly inclined bottom or floor 4 which is common to the two chambers 5 and 6 of the furnace, which in turn 10 are formed by a partition wall 9 extending downwardly from the arched roof portions 7 and 8 disposed above the two chambers of the furnace, the partition extending to a point which is sufficiently spaced from the floor 4 to allow of free 15 passage of metal from one portion of the chamber to the other and also to permit of a rapid and free interchange of heat from the material in the chamber 5 to the material in the chamber 6. As an aid to the passage of heat from one 20 said chamber to the other the partition 9 may be formed of a refractory material of relatively high conductivity.

The chamber 5 of the furnace serves as a 25 chamber in which heat is applied to melt the metal and to maintain metal in molten condition and is provided with a curved inner wall 10 (see Fig. 3) to reduce to a minimum the loss of material through the formation of oxides or the lodging of dross or foreign material in corners, 30 which has been an objectionable feature in many furnaces of this type. This chamber 5 is provided with an opening in its outer wall above the level of the bath to be maintained therein, which is normally closed by means of a door 12 35 connected with a counterweight 13 for convenient operation. It is also provided with a fuel inlet port 14, through which any suitable fuel, such as oil, gas or other material may be introduced into the upper portion 15 of the chamber 40 box where the burning fuel will supply heat directly to the surface of the molten bath of material in the chamber. A small passage 16 extends through the partition wall 9 and allows products of combustion to flow into the upper 45 portion 17 of the chamber 6. The products of combustion of the fuel burned in the space 15 will discharge by leakage around or past the door 12 and only a small amount of gas will pass through the passage 16 into the chamber 17.

50 The second chamber 6 is similar to the first chamber in general form, but is provided with an outer wall 18 of considerable slope to permit of convenient removal of chunks of iron or foreign material which may accidentally be charged into 55 this chamber and which may then be removed by raking or by electro-magnetic means, the inclined wall 18 serving as a slope against which such material may be removed. At the top of the inclined wall 18 is a door 20 connected to a suitable counterweight 21 for convenient operation, this door normally closing an opening in the wall of the furnace, through which access may be had when necessary to the interior of the furnace chamber. The upper or dome-like roof 60 of the chamber 6 is provided with a vent or stack 21, which permits the discharge of excess gas from the upper portion of the chamber, and is also provided with a charging port 22, which is best shown in Fig. 2. The charging port 22 65 forms the end of a slightly inclined passageway 23, in which there is mounted a piston 24, operated when desired by a rod 25, crank 26 and handle 27. The passageway 23 is provided with an opening 28 communicating with a hopper 29, 70 into which finely divided material to be melted

75 is supplied, and from this hopper the material flows down onto the inner wall or ledge 30 of the passageway 23, where it is preheated to a point slightly below its melting point by the temperature of the atmosphere which is maintained on top of the bath in the chamber 6. The charge ordinarily carried on this ledge 30 is then forced off from the ledge and allowed to drop into the molten bath whenever desired by operating the charging piston 24 by means of a crank 27. At 10 all times, however, this exit from the chamber 17 is sealed either by the charging piston 24, when in the position shown in Fig. 2, or by the material resting on the ledge or bottom of the passageway 23 when the piston is retracted. 15

Agitating means for the purpose presently to be described are provided in the form of a shaft 35, slidably and rotatably mounted in a bracket or carrier 36, which in turn is supported by means of a fluid pressure cylinder 37 from a trolley 38 which is movable horizontally along a trackway 39. Movement of the trolley 38 and agitating means carried thereby in a direction along the trackway away from the furnace will cause actuation of a switch 40, opening the circuit of the motor 40 and causing cessation of the operation of the agitating mechanism. A return of the trolley and other parts to the position shown in Fig. 1 will also automatically close the switch and reestablish the circuit. Also carried on the bracket 36 is a motor 40 provided with a worm 41 driving a worm gear 42 which is slidably but non-rotatably mounted on the shaft 35 so that rotation of the motor 40 causes rotation at predetermined speeds of the shaft 35. 35 On the lower end of the shaft is mounted an agitating mechanism having a series of irregularly arranged and spaced arms 45, which are preferably of different lengths for reasons to be presently described. At the upper end the shaft is provided with a free handle 46 for convenient manipulation, while intermediate its ends it may be provided with a more or less spherical enlargement 47 formed of suitable refractory material and roughly fitting into a suitable opening 49 in the door 20 to permit of manipulation of the agitating means in the chamber by operation of the handle outside of the chamber. 45

At the base of the furnace, pouring spouts 50 and 51 are provided (see Fig. 2) for pouring 50 the molten material when desired, either into ladles or directly into the molds, the openings being normally closed by plugs of refractory material in the usual manner. Also at the lower point of the floor of the furnace there is an 55 opening 53, through which the furnace may be cleaned at intervals, this opening normally being closed by a permanent plug.

My improved furnace is initially placed in operation by charging pieces of aluminum into the 60 furnace, melting these to produce a bath of material sufficient to rise above the top of the opening connecting the two chambers 5 and 6, above the bottom of the partition 9. Thereafter finely divided material may be charged into the furnace 65 by the charging piston 24 in sufficient quantities and at sufficient intervals to compensate for molten material which is withdrawn as required for casting into ingots or other articles. The heat for melting the initial charge, and also the 70 continuing charges, is supplied through the fuel inlet 14 and the fuel burns in the space 15 above the chamber 5. A small amount of burning fuel passes through the port 16 into the space 17 above the chamber 6 and the burning of this fuel 75

in the space 17 burns out the oxygen in this space, leaving an inert, non-oxidizing atmosphere above the bath in the chamber 6. Additional products of combustion leak from the 5 space 15 to the space 17 and any excess gas in the latter space is allowed to discharge through the vent 21.

The material in the chamber 6 is heated by conduction through the partition wall 9 and also 10 by conduction through the metal connecting the baths in the two chambers 5 and 6 and possibly, to some extent by some type of thermo-siphonic circulation through the molten material.

After the furnace has been placed in operation 15 and a bath of appreciable depth secured, further operation of the apparatus and of the process is as follows. A charge of finely divided aluminum is first allowed to pass from the hopper on to the ledge 30, where it is preheated by 20 the gaseous contents of the chamber 17 to a temperature which approximates the heat-treating temperature of aluminum, which is a temperature which approaches but does not reach the melting temperature of the material. This 25 nearly molten charge is then pushed from the ledge into the bath by the piston 24. The finely divided material falls upon the surface of the bath, passing through any coating of dross thereon, and is gradually absorbed into the bath by melting, this absorption being relatively rapid because of the elevated temperature of the newly charged material. During this part of the operation 30 the agitating means may be rotated either very slowly or not at all until the charged solid 35 material has become molten and is mixed with the bath, and it is desirable to have a minimum of agitation at this stage as otherwise too thick a layer of dross is formed on top of the bath, which tends to hinder entrance of the new material 40 into the bath proper. After absorption into the bath, however, of the new charge the agitation is increased in speed as rapidly as possible until a blade speed is secured of approximately 700 feet per minute.

45 It will be understood that suitable fluxes, the nature of which should be dependent upon the analysis of the materials employed, are included in the bath being charged with the aluminum or separately as may be found most suitable. Also 50 the material charged into the bath should preferably be partially cleaned before charging to remove as much as possible of the dirt, oil and grease which is ordinarily inseparable from fine material of the type referred to. A certain 55 amount of such material, however, will inevitably be included with the charge and will be agitated and burned upon the surface and above the surface of the bath. The burning of this material will occupy but a short time and will 60 leave the upper portion 17 of the chamber 6 with a non-oxidizing or inert atmosphere in contact with the surface of the bath and with the material waiting to be charged upon the ledge beneath the hopper. By thus removing the active 65 combustion and heating from that portion of the furnace in which material is charged I avoid the very rapid oxidation of such material and the consequent loss of material and increased time and effort required to clean it which is inevitable in the types of remelting furnaces heretofore used.

From the foregoing description it will be evident 70 that my method of melting finely divided aluminum consists in maintaining two connecting baths 75 of the material, charging pre-heated solid mate-

rial into one of the baths while transmitting heat from the other of the said baths through the intervening partition and the intervening mass of metal into the bath into which the newly charged material is received. The apparatus described is constructed to facilitate the effective carrying out of this method. The chamber 5 is formed of roughly frusto-conical shape, affording a large surface to the bath, to which heat is imparted from the upper portion of the chamber. In this way a maximum amount of heat can be transmitted into the bath and then transmitted through the bath to the connecting neck of metal lying beneath the partition wall 9. By constructing a partition wall of relatively conductive material a large amount of heat can also be transmitted directly through this wall. At the same time the atmosphere above the bath in which the finely divided material is being pre-heated and subsequently absorbed into the bath 10 is maintained in an inert condition, thus preventing the rapid oxidation of this material, which has been a difficulty in most types of furnaces for the remelting of fine material.

The agitation given to the material is of prime 15 importance. During the stage when new material is charged into the bath in chamber 6, or when this newly charged material is being melted and absorbed into the bath the latter should be agitated as little as possible, as otherwise the full 20 absorption of the newly charged material is prevented. As soon, however, as the bath in the chamber 6 is fully molten the agitating means are operated vigorously and rapidly, being directed throughout the bath by the attendant who 25 controls the operation from outside of the furnace, making it possible to operate upon every portion of the bath in an irregular and unrhythmic manner which does not set up continuous 30 rhythmic streams of material, but breaks and tears apart the material throughout the bath by churning, striking and violently agitating all of 35 this molten material. The agitation of the material in this manner in conjunction with the flux 40 has a result of reducing the surface tension of the mass, loosening what may be termed the bond between the particles of clean metal and unclean metal, permitting the entrained and occluded gases to be freed from the material. This 45 action is continuous and relatively uniform 50 through the entire bath where the action of the irregularly operated agitating means ruptures the surface skin tension of the material at every point, and the agitating arms then literally break loose the foreign matter from the pure metal, 55 causing the foreign material to rise to the surface of the liquid in the form of dross. By maintaining a very rapid, violent, but irregular action of the agitating means I have found it possible to 60 free molten metal entirely of its foreign material 65 without carrying any appreciable amount of pure metal to the surface with the foreign material. It will of course be evident that one source of loss in the operation of such a furnace is the removal from the mass of material of some pure metal along with the dross, and in many furnaces this 70 is a source of heavy loss.

The layer of dross on top of the bath may of course be raked through door 20 whenever the accumulation becomes excessive and interferes 75 with the passage of finely divided charge into the bath proper, but until it becomes excessive this layer of dross acts as a protective coating, sealing the bath from even the inert atmosphere above it and insuring against oxidation of the molten 75

metal by any stray currents of oxidizing gas which may drift into the upper portion of the chamber 6 from the heating chamber 15.

The material thus purified can be drawn off at 5 intervals through the spouts 50 and 51 into suitable molds to form either ingots or cast articles of any desired shape, and, treated as above described, the metal thus drawn off is relatively pure and of high enough quality to make it unnecessary to include any subsequent cleaning operation, as is invariably the case with furnaces now in use in which the metal is drawn off into ladles, which are then agitated by attendants with rakes to complete the removal of the foreign 10 material. For production of ingots I have devised molds, which are shown in Fig. 2, and which will now be described.

My improved molds consist of horizontal elements 60 (see Fig. 2) provided with recesses 61 separated from each other by full height partitions 62 and by low partitions 63 which permit the two ingots formed in each of the two partially formed chambers to be connected but still capable of being broken apart either upon cooling or with 15 very little effort by the user. The chambers 61 are fed by sprues 64 at the ends, which connect with sprue 65 branching from a main pouring sprue 66 which is formed in the end plate 67 of the mold assembly shown in Fig. 2. In assembling the molds a base 68 is first employed, after 20 which a series of molds 60 are mounted in registration with each other upon the base, and the end plates 67 are applied and clamped in position by means of straps 69 extending around the side 25 of the mold box from one end plate to the other, where they are tightened by means of cams 70 and handles 71.

By forming the molds in this manner and grinding to a true surface all of the contacting 30 surfaces of the base, mold and end plates it is possible to clamp the assembled parts together in such a way as to provide perfectly tight pouring sprues between the parts, take advantage of the shrinkage of the metal in cooling to break apart 35 the ingots from each other and to provide a mold of long life which is easily assembled and disassembled.

Other forms may be employed embodying the features of my invention instead of the one here- 40 in explained, change being made in the form or construction, provided the elements stated by any

of the following claims or the equivalent of such stated elements be employed, whether produced by my preferred method or by others embodying steps equivalent to those stated in the following claims.

I therefore particularly point out and distinctly claim as my invention:—

1. In a method of melting finely divided aluminum, the steps which consist in maintaining two connected baths of molten aluminum, heating 10 one of said baths, transmitting a portion of the heat imparted to the first-named bath to the other of said baths, maintaining a substantially inert atmosphere in contact with the second of said baths, charging into the last named bath a 15 quantity of pre-heated aluminum, slowly agitating said bath during absorption of such charge thereto, and then violently agitating said bath to clean the molten aluminum therein and to cause the separation of all foreign material from 20 the aluminum.

2. In a method of melting finely divided aluminum, the steps which consist in maintaining two connected baths of molten aluminum, imparting heat to one of said baths, conducting part of 25 the heat imparted to said bath to the other of said two baths, maintaining a substantially inert atmosphere in contact with the second of said baths, preheating a charge of finely divided aluminum in such inert atmosphere over said second 30 bath to a temperature slightly below the melting point, charging such preheated aluminum into said second bath, slowly agitating said bath until the said charge is absorbed thereto in molten 35 condition, and then agitating said bath violently to separate foreign material from the aluminum.

3. In a method of melting finely divided aluminum, the steps which consist in maintaining two connected baths of molten aluminum, heating one of said baths by means of fuel burned above 40 said bath, transmitting a portion of the heat imparted to said first-named bath to the other of said baths, transmitting a portion of said burning fuel to the space above said second bath so as to maintain a substantially non-oxidizing atmosphere in contact with said second bath, and violently agitating said last-named bath to clean the molten aluminum therein and to cause the separation of all foreign material from the aluminum.

LOUIS O. GARWIN.